

June 10, 1930.

H. CLAUSER

1,762,911

SEALING COMPOUND FOR PYROTECHNIC DEVICES

Filed Feb. 2, 1926



Inventor

By *Herbert Clauser*,  
*Watson, Coit, Moore & Grindell*

Attorney

Patented June 10, 1930

1,762,911

## UNITED STATES PATENT OFFICE

HERBERT CLAUSER, OF ELKTON, MARYLAND, ASSIGNOR TO VICTORY SPARKLER &amp; SPECIALTY COMPANY, OF ELKTON, MARYLAND, A CORPORATION OF DELAWARE

## SEALING COMPOUND FOR PYROTECHNIC DEVICES

Application filed February 2, 1926. Serial No. 85,592.

This invention relates to pyrotechnic devices or fireworks and consists in a novel composition for sealing the same to confine the gas generated by explosion or combustion.

I have chosen, as an example of the use of my improved sealing material, the firework known as a "toy torpedo" or "tube torpedo", and have shown such a device in 10 the drawing, in which:

Fig. 1 is an elevation of a tubular toy torpedo;

Fig. 2 is a central vertical section of the same; and

15 Fig. 3 is a plan view thereof.

In these views, A is the container or tube, of paper, cardboard, or the like; B is a cup of the same material inserted in the lower end of the tube; D is the explosive composition placed in and on said cup; E is the gravel or other detonating medium; C is a disk of cardboard fitted in the tube on top of the charge, and F, F represents the sealing material in the extreme ends of the tube.

20 Many materials and compositions have been tried and used for sealing fireworks of this type, but none of them, as far as I am aware, has proved entirely satisfactory, either from the standpoint of its manufacture or of its behavior under varying climatic conditions.

25 My improved composition obviates all the defects heretofore existent in the materials used for the purpose in question. For instance, it does not require an excessive time for drying; it does not crack after being dried; it does not expand or contract in unequal relation to the other parts of the device; it does not shatter upon the impact 30 necessary to explode the torpedo, before the explosion takes place, and, when shattered, the flying pieces cannot do any harm or injure anyone. Further, it is waterproof and fireproof.

35 The preferred composition of my improved sealing material is as follows: silicate of soda 50 lbs.; kaolin 40 lbs.; zinc oxide 9.5 lbs.; and coloring material 0.5 lbs. The latter may be ultramarine blue, vermillion red, or the like, and may, of course, be

omitted. The kaolin is a filler and, obviously, other fillers may be used, such as fuller's earth, filter-cel, and the like. Also, in place of zinc oxide, other metal oxides, such as those of magnesium, lead or iron, 55 may be used.

This composition partially sets very quickly, thus facilitating its transport from one department of the factory to another, and finally sets more quickly than the compositions heretofore used.

The above proportions of the ingredients have proved very satisfactory, but I do not wish to limit myself to them.

Having thus described my invention, what 65 I claim to be new and desire to secure by Letters Patent is:

1. A material for sealing fireworks comprising a mixture of substantially 50% of silicate of soda, substantially 10% of a metallic oxide and substantially 40% of silicate of alumina.

2. A material for sealing fireworks comprising a mixture of substantially 50% of silicate of soda, substantially 10% of zinc 75 oxide and substantially 40% of kaolin.

In testimony whereof I hereunto affix my signature.

HERBERT CLAUSER.

80

85

90

95

100